

United States Patent [19]  
Darnell et al.

[11] 3,870,513  
[45] Mar. 11, 1975

[54] WHITE METAL CASTING ALLOY AND  
METHOD OF MAKING SAME

[75] Inventors: Robert S. Darnell, Washington, R.I.;  
Everett G. Morrissey, Bristol, Mass.

[73] Assignee: A. J. Oster, Co., Providence, R.I.

[22] Filed: Dec. 3, 1973

[21] Appl. No.: 420,948

[52] U.S. Cl..... 75/175 A

[51] Int. Cl..... C22c 13/00

[58] Field of Search..... 75/175 A, 175 R

[56] References Cited

UNITED STATES PATENTS

|           |         |                    |          |
|-----------|---------|--------------------|----------|
| 2,097,727 | 11/1937 | Hanson et al.....  | 75/175 A |
| 2,180,139 | 11/1939 | Deitz.....         | 75/93    |
| 2,303,193 | 11/1942 | Bouton et al. .... | 75/166   |
| 2,891,511 | 6/1959  | Fehling .....      | 120/42.4 |

3,563,732 2/1971 Morisaki..... 75/175 A

Primary Examiner—L. Dewayne Rutledge

Assistant Examiner—E. L. Weise

Attorney, Agent, or Firm—Salter & Michaelson

[57] ABSTRACT

A white metal casting alloy comprising as its essential ingredients tin, antimony, cadmium and lead in specified proportions. The invention further comprises a method of making said alloy comprising the steps of mixing a certain amount of the tin to be used with the lead and the antimony at a temperature of approximately 800° F. until the antimony is dissolved and then adding the remaining amount of the tin and mixing until the alloy becomes homogenous, and then cooling the mixture to approximately 475° F., at which point the cadmium is mixed and dissolved.

3 Claims, No Drawings

# WHITE METAL CASTING ALLOY AND METHOD OF MAKING SAME

## BACKGROUND AND SUMMARY OF THE INVENTION

The present invention relates to casting alloys of the type frequently used with centrifugal rubber molds, such as during the casting of jewelry and similar products. Alloys of this type embodying a high tin composition are known in the trade as white metal alloys, and such alloys must generally meet the following requirements. First of all, the cast alloy must lend itself to a high degree of polishing. Secondly, the cast alloy must be capable of being effectively and efficiently plated. The cast alloy must not be excessively brittle, since the cast articles, particularly where designed for jewelry use, frequently embody prongs that must be bendable. In addition, it is desirable that the alloy be capable of being cast at as low a temperature as possible, since the lower the casting temperature, the longer the life of the molds, particularly where of rubber construction. In addition, the casting alloy must have good flowability.

White metal alloys, by definition, comprise a high tin content, generally upwards of 90% by weight. It is quite conventional to alloy antimony with tin, since the antimony adds a desired degree of hardness to the alloy, without unduly or adversely affecting the castability of the tin. For example, one of the more conventional prior art alloys of this type is a product of American Smelting & Refining Co. and is called "OR-8" and comprises 92% tin and 8% antimony. Other prior art alloys, in addition to tin and antimony, may also comprise lead in order to increase the flowability of the alloy, or copper, in order to increase the strength of the alloy. Examples of such prior art compositions are alloys comprising 94.5 parts tin, one part antimony, and 4.5 parts lead; or 92 parts tin, 4 parts antimony, and 4 parts lead; or 90.5 parts tin, 7.5 parts antimony, and 2 parts copper.

Although prior art alloys of the type above mentioned have proven to be generally satisfactory for their intended purposes, it has nevertheless been found that an alloy comprising as its essential ingredients tin, antimony, cadmium and lead, in proportions hereinafter to be specified, produces unexpectedly good results. As previously stated, the tin in the composition permits the alloy to be cast, while the antimony adds desired hardness thereto. The presence of lead increases the flowability of the alloy and helps to prevent undesirable shrinking of the cast alloy during cooling. The presence of cadmium appears to make the alloy more ductile and bendable and at the same time lowers the temperature at which the alloy may be cast. More specifically, conventional prior art white metal alloys will normally be cast at a temperature of 650° - 700° F. The alloy of the present invention, on the other hand, may be cast at a temperature of 500° - 550° F. This lower casting temperature is a pronounced advantage, since it promotes longer mold life, particularly where the molds are of rubber construction. In addition to the advantages just stated, the alloy of the present invention has all of the other necessary characteristics of a good casting alloy, i.e., readily lends itself to high polishing, is capable of being effectively plated, and has good flowability. In fact, the present composition appears to be more effec-

tive in these respects than the conventional prior art white metal casting alloys.

## DESCRIPTION OF THE INVENTION

5 In carrying out the present invention, it has been found that an alloy comprising 90.5 - 92.5% tin, 2.9 - 3.1% antimony, 1.4 - 1.6% cadmium, and 3.3 - 3.7% lead achieves the advantageous results hereinbefore discussed. Preferably, the alloy comprises 92% tin, 3% 10 antimony, 1.5% cadmium, and 3.5% lead. It is important to note that since cadmium adds toxicity to the alloy, an excessive amount (over 5%) would be detrimental. In lesser amounts, however, i.e., approximately 1.5% of the alloy, the presence of the cadmium is not 15 only not detrimental, but appears to be highly desirable in that it adds to the ductility of the alloy and at the same time lowers the casting temperature thereof. In addition, it has been found by chemical analysis that the alloy of the present invention has a unique crystalline structure of its own, which can be described as true crystalline, in comparison with the amorphous structures of OR-8, which indicate a two-phase eutectic alloy. This is thought to be attributable to the presence 20 of cadmium in the composition.

25 In making the present composition, the lead and antimony are mixed with 75% of the tin to be used at a temperature of approximately 800° F. until the antimony dissolves, at which point the other 25% of the tin is added to the mixture and is homogeneously dispersed 30 therein, as by conventional mixing apparatus. After the mixture has become homogenous, it is allowed to cool until it reaches a temperature of 475° F. or slightly lower, at which point the cadmium is added and mixed 35 therein until dissolved. The alloy is now ready for casting and, as previously stated, may be cast and formed at temperatures of 500° - 550° F.

Also of importance is the purity of the metals used. Thus, the tin should be 99.891% pure, while the cadmium should be 99.99% pure and the lead 99.9% pure 40 in order to obtain the most desirable results.

In addition to the hereinbefore discussed advantages of the present alloy, it has additionally been found that it is possible to plate gold by immersion onto the alloy. More specifically, the system used was a gold plating solution known commercially as Tivaklad GI-3 sold by Tivian Laboratories, Inc., of Providence, Rhode Island. It consists of a buffered gold chelate having the following composition:

|             |              |
|-------------|--------------|
| Gold        | 1 troy ounce |
| Chelate     | 2 pounds     |
| Water       | 1 gallon     |
| pH          | 3.0          |
| Temperature | 140-150° F.  |

50 The capability of the present alloy to be gold plated by immersion is a completely unexpected result and constitutes a further advantage of the present alloy, since gold plating by immersion has not heretofore been possible with conventional prior white metal casting alloys.

55 As this invention may be embodied in several forms without departing from the spirit or essential characteristics thereof, the present embodiment is therefore illustrative and not restrictive, since the scope of the invention is defined by the appended claims rather than by the description preceding them, and all changes that fall within the metes and bounds of the claims or that

form their functional as well as conjointly cooperative equivalents, are therefore intended to be embraced by these claims.

What is claimed is:

1. A white metal alloy consisting of 91.5 - 92.5% tin, 2.9 - 3.1% antimony, 1.4 - 1.6% cadmium, and 3.3 - 3.7% lead.

2. The alloy of claim 1 further characterized in that said tin is at least 99.891% pure, said cadmium is at least 99.99% pure, and said lead is at least 99.9% pure. 10

3. The method of making the alloy of claim 1, comprising the steps of mixing together at approximately 800° F. the lead, the antimony and approximately 75% of the tin until the antimony has dissolved, then adding the remainder of the tin to the mixture and mixing same until the mixture has become substantially homogeneous, then causing the mixture to cool to 475° F. or slightly less, then adding the cadmium and mixing until the latter has dissolved.

\* \* \* \* \*

15

20

25

30

35

40

45

50

55

60

65